

1,418,514.

L. BAILEY.  
CONCENTRATION OF ORES.  
APPLICATION FILED NOV. 9, 1917.

Patented June 6, 1922.

2 SHEETS—SHEET 1.



L. BAILEY.  
CONCENTRATION OF ORES.  
APPLICATION FILED NOV. 9, 1917.

1,418,514

Patented June 6, 1922.

2 SHEETS—SHEET 2.

FIG. 4



Inventor:  
Lewis Bailey  
by Arthur P. Knight  
his Attorney

# UNITED STATES PATENT OFFICE.

LEWIS BAILEY, OF HAYDEN, ARIZONA, ASSIGNOR TO MINERALS SEPARATION NORTH AMERICAN CORPORATION, OF NEW YORK, N. Y., A CORPORATION OF MARYLAND.

## CONCENTRATION OF ORES.

1,418,514.

Specification of Letters Patent. Patented June 6, 1922.

Application filed November 9, 1917. Serial No. 201,062.

To all whom it may concern:

Be it known that I, LEWIS BAILEY, a citizen of the United States, residing at Hayden, in the county of Gila and State of Arizona, have invented a new and useful Improvement in Concentration of Ores, of which the following is a specification.

This invention relates to concentration of ores of copper and other metals by the process of flotation, wherein a body of pulp consisting of finely divided ore and water, is aerated so as to form bubbles therein, suitable flotation agents, such as oil, tar, etc., being used to cause the mineral of the ore to be selectively floated by the bubbles as they rise to the surface of the body of pulp, and to be thereby separated from the gangue of the ore.

The main object of the present invention is to apply the flotation agent aforesaid in the most effective and economical manner, and particularly to so apply said agent that it will be uniformly supplied to all parts of the pulp.

Another object of the invention is to dispense with any agitation of liquid flotation agent such as oil or tar, with the pulp, thereby simplifying and reducing the cost of the process and of the apparatus used for carrying it out and also increasing the efficiency of the process.

In concentrating ores by flotation, it has generally been considered necessary to agitate the oil or other flotation agent with the pulp to secure efficient selective action of the flotation agent with respect to the mineral and gangue constituents of the ore, and in such agitation, the flotation agent, often in masses or globules of considerable size, was brought forcibly into intimate and prolonged contact with the gangue particles, with the result that such particles were liable to become more or less coated with such agent, notwithstanding the selective action of the latter, and the gangue so coated was carried along with the mineral values, so that the resulting rougher concentrates required much cleaning. An important object of the present invention is to more effectively prevent such prolonged contact of liquid, oil, etc., with the gangue particles and to correspondingly reduce the amount of gangue material carried along with the mineral values and the amount of recleaning needed on the rougher concentrates.

The above recited objects, as well as other

advantages hereinafter referred to, are attained according to this invention, by supplying the oil, tar or other flotation agent, in the form of a vapor mixed with the air or other gas used for aeration, and by so applying this mixture of vapor and gas to the body of pulp that the resulting bubbles are uniformly distributed in the pulp, and the flotation agent is presented to the pulp at the surfaces of such bubbles, the operation being carried on in such manner that there is no opportunity for flotation agent to collect in liquid form, in masses of any considerable size, in the pulp.

My invention may be carried out in any suitable apparatus adapted to supply the flotation agent in the form of vapor mixed with air or other gas, and to apply such mixture of vapor and gas to the pulp in such manner as to form bubbles distributed uniformly through the body of pulp, said bubbles ascending through the pulp and conveying the flotation agent to all parts of the pulp with substantial uniformity. The apparatus shown in the accompanying drawings is, however, especially adapted for carrying out the process. Referring to said drawings:

Fig. 1 is a partly sectional side elevation of such flotation apparatus.

Fig. 2 is a partial plan view thereof.

Fig. 3 is a partial vertical section, showing two of the flotation cells.

Fig. 4 is a section on line 4—4 in Fig. 1.

In carrying out my invention, I prefer to use flotation cells of the form shown at 1 in Figs. 3 and 4, comprising side walls 3, vertical partition walls 4, and a floor 5, said floor being inclined to facilitate flow of pulp thereover and the partition walls 4 being spaced from said floor to permit flow of the pulp from cell to cell. Suitable baffles 6 are provided for regulating such flow, said baffles being, for example, mounted for vertical adjustment, by screw rods 7, engaging in hand wheels 8, which rest on top bars 9. Of the two cells shown in Fig. 3, the first or uppermost cell 1 is adapted for supply of the flotation agent along with air, the floor of said cell being provided with a passage or chamber 10, connected to suitable means for supplying a mixture of air and of flotation agent in the form of vapor, the top of said chamber being formed of a porous mat or plate 11, over which the pulp flows. Said cell 1 may also be provided

with a chamber or chambers 12 in its floor, covered by a porous mat or plate 13 and communicating with a source of compressed air. The mat or section of the floor through which the mixture of flotation agent and air is admitted is preferably located at the upper end of the cell. Any desired number of cells, such as shown at 1 in Fig. 3, may be arranged in series so that the pulp 10 will flow through all of them successively, and in addition there are preferably provided cells of the form shown at 2 in Fig. 3, said cells 2 being of similar construction to cell 1, except that the air supply 15 passages 15 in the bottom thereof, are connected only to compressed air supply means for furnishing air for aeration of the pulp through porous mats or plates 16, between said passages and said cells. I have found 20 it advantageous to make the floor sections or porous mats or plates 11, 13 and 16 of molded material, such as porous cement composition, consisting, for example, of quartz or rock screenings bonded with Portland 25 cement, the screenings for sections 11 being, for example, of about 6 to 8-mesh size, and the screenings for sections 13 and 16 being, for example, of about 20-mesh size, so that the sections 13 and 16 are of closer or finer 30 grained structure than the sections 11. Only a small amount of cement is used (say one part cement to five of rock screenings), and only sufficient water is used to cause the cement to coat the rock particles and cause 35 same to adhere to one another, leaving multitudes of pores or interstices between said particles, and also leaving the surface of the particles in rough condition so that even where the particles are in contact, the 40 contiguous surfaces are so rough and porous that minute interstices are formed therebetween, giving extreme sub-division to the air.

The flotation cells constructed as above 45 described, may be arranged in series in any suitable manner, to receive the pulp successively in the series of cells. The arrangement of cells shown in Figs. 1 and 2 is advantageous, in that it provides for continuous gravity flow of the pulp through 50 all the series of cells, and dispenses with any return or circulation of the pulp, and therefore, with the pumping means that would be required for such circulation.

55 The apparatus shown in the said Figs. 1 and 2, comprises a series of rougher cells 1 and 2, adapted to receive the pulp from suitable feed or supply means 17, a series of cleaner cells 18, adapted to receive the 60 rougher concentrates from the rougher cells 1 and 2, and cleaner cells 19, adapted to receive tailings from cleaner cells 18, the concentrates from series of cells 18 and 19 discharging into a concentrates launder 20, by 65 which they are conducted to dewatering

means in usual manner. The ore pulp supply means 17 comprises a chute delivering the pulp into a receiving chamber 21, from which the pulp flows over a baffle 22 into the bottom part of the first cell of series 1, in 70 such manner that any agitation of the pulp is avoided. From the lower ends of the series of rougher cells, the rougher tailings pass to tailings launder 26. The tailings from cells 19 pass off through tailings 75 launder 27.

The compressed air supply means may comprise an air pump 28 adapted to compress air to a pressure of about 1 to 6 pounds, preferably about two pounds, to the square 80 inch, and a pipe 31 connected to receive the compressed air from said pump and leading to a chamber or receiver 30 having outlet pipes 32 leading to the passages 10 of the several cells 1, valves 33 being provided 85 in pipes 32 for controlling the flow of air to each of said cells. Suitable means are provided for supplying flotation agent, such as a flotation oil, to the air passing to chamber 30. For this purpose, a tank 36 containing such agent in liquid form, is connected by piping 37, including a needle valve, to a high pressure compressed air pipe 39 leading to an atomizer 38 which sprays or atomizes the liquid flotation agent into pipe 31. 95 The high pressure air, which may be at any pressure suitable for the atomizing operation, may be supplied by a pump 40. This high pressure air may also be conducted from pump 40 by pipes 42 and 43 to the top 100 of oil tank 36 and to the top of upper supply tank 44, which feeds tank 36 through pipe 45, it being understood that in an installation of considerable size, the tank 44 may feed several tanks 36 corresponding to 105 different units. By opening a valve 47 in pipe 45, the tank 36 may be filled without stopping the operation, as the same air pressure is maintained in both tanks. A drain connection 50, provided with a valve 51, 110 leads from each chamber 10 to a sump 52, so as to enable any liquid such as condensed oil, collecting in chamber 10 to be drawn off therefrom, said liquid being pumped back to tank 44, if desired, by pump 55. 115

An air main 57 is connected to air pump 28 and valved pipes 60 lead from said main to respective air supply passages 12 and 15 of the rougher cells 1 and 2. Extensions 58 and 59 of air main 57 are connected by 120 valved pipes 63 to the air supply passages for the cleaner cells 18 and cells 19.

Other apparatus than that above described may be used for carrying out my invention, provided it is adapted to apply the mixture 125 of air vapor of oil or other flotation agent to the pulp with the required degree of uniformity, and to provide the necessary aeration of the pulp to complete the flotation. In particular, the porous mats or plates 130

through which the air is forced, may be of various materials, whether natural porous rock, or artificial slabs of any kind, it being necessary, however, that these mats should 5 be porous, and of considerable extension so as to present a multiplicity of closely spaced openings extending over a sufficiently large surface to provide for uniform distribution of the air in the pulp.

10 My process may be carried out in the above described apparatus, as follows:

The ore pulp, resulting from comminution of the ore with water, is conducted by feed means, to the upper end of the series 15 of rougher cells, without any preliminary agitation or treatment with oil or other flotation agent, and flows successively through all of said cells. Air, compressed by pump 28 to a pressure of say, four to five pounds 20 per square inch, is conducted through pipe 31 wherein it is charged or impregnated with a flotation agent distributed thereto by atomizer 38. Any suitable oil or other flotation agent may be used, provided it is 25 of sufficient volatility to enable it to be vaporized and carried forward by the air (or at least to enable a sufficient portion thereof to be vaporized for the purpose of this invention). If the flotation agent is not sufficiently volatile to enable it to be vaporized 30 by atomization into the air passing through pipe 31, it may be vaporized by heat applied in any suitable manner—for example, by heating the air into which it is supplied, such heating of the air not being herein 35 specifically claimed by me. The mixture of air and vaporized flotation agent passes to chamber 30, whence it is distributed by pipes 32 to the several passages or chambers 10 in 40 the floor or bottom of cells 1, and passing up through the pores or interstices of the porous mats or plates 11, issues therefrom in the form of jets or streams of vapor laden air. Such air, on entering the pulp, breaks 45 up into bubbles which rise in the pulp, and by reason of the great number, close spacing and variant direction of the streams of air (due to the irregular porous structure of the mats or plates 11), the whole body of pulp 50 above the said mats or plates 11, becomes filled or occupied with substantial uniformity, by bubbles of air carrying flotation agent. The flotation agent is applied to, or comes in contact with the pulp particles at 55 the surfaces where the bubbles adjoin such particles and when so applied, it is in the form of most minute sub-division, so that no agitation is required or used, either for subdividing the oil or other flotation agent, or 60 for distributing it in the body of pulp, the required sub-division resulting directly from the contact of the vapor laden air with the pulp, and the required distribution resulting from the uniform distribution of the 65 bubbles in the pulp. In fact, the sub-divi-

sion and distribution of the flotation agent by this method may be made more effective than is practicable by agitation of liquid oil with the pulp. While it is the aim of this invention to apply the flotation agent mainly 70 in the form of vapor, there may, under certain conditions, be more or less of the flotation agent carried along in the state of fine particles of liquid suspended in the air and vapor.

In addition to its function of supplying the flotation agent in condition of extreme sub-division and at the same time distributing such finely divided agent to all parts of the pulp, the compressed air forced into the 80 lower part of the cells 1, as above described, serves as an aerating agent for the pulp, the bubbles produced in the pulp by the air, rising to the surface and flowing over the side walls 3 of the cells, this overflowing foam or 85 mass of bubbles carrying with it the concentrates which pass along the launders 20 to the cleaner cells. The complete operation of the air supplied in this manner and laden with vapor of flotation agent so as to distribute oil or other flotation agent to the pulp, as well as to aerate the same, may be termed an oiling aeration, as it performs both of these functions simultaneously, the word "oiling", in this case, including the use 90 of any equivalent flotation agent capable of being supplied by the air in this manner. In practice, I find it desirable to introduce a further amount of air for aeration purposes only, in addition to that supplied for oiling 100 aeration as above described. In the apparatus shown in the drawings, this additional aerating air is introduced partly in the same cells 1 that are used for the oiling aeration, and partly in succeeding cells 2, which are 105 used for aeration only. Air under a pressure of say, 1 to 6 pounds, (preferably about 2 pounds) per square inch, passes from main 57 through valved pipes 60 to the several passages 12 below the respective porous plates 13 of cells 1, and to passages 15 below the respective porous plates 16 of cells 2, so that minute bubbles of air are disseminated throughout the pulp in all the cells, and in rising through the pulp, carry up 110 with them the mineral concentrates thereof, so as to complete the flotation of the concentrates from the pulp. I have shown the first three cells 1 in each row as provided with means for oiling-aeration, and the remaining cells 2 of each row as provided with means for aeration without further supply of oil, etc., but the means for oiling-aeration may be provided in any desired number of the series of rougher cells, and even in some 115 of the cleaner cells. It will generally be sufficient, however, to provide the series 18 of cleaner cells, and the cells 19 with the compressed air connections only, as indicated at 63.

What I claim is:

1. The process of concentrating ores, which consists in first subjecting a pulp of comminuted ore and water, to oiling aeration by distributing therein, air containing oil vapor, and then to further aeration by distributing air alone therein.
2. The process of concentrating ores, which consists in forcing into a flowing pulp of comminuted ore and water, air carrying a flotation agent, so as to distribute flotation agent in the pulp, and forcing into the pulp in which flotation agent has thus been distributed, a further quantity of air alone for completing flotation of mineral in the ore.
3. An apparatus for ore flotation, comprising a cell provided with means for passing ore pulp therethrough, a plurality of passages adjacent to the lower part of said cell, porous plates between said passages and the cell, means for supplying compressed air mixed with vapor of flotation agent to one of said passages, and means for supplying compressed air alone to the other of said passages.
4. An apparatus for ore flotation, comprising a series of cells connected to successively receive ore pulp, means for applying and distributing gas carrying flotation agent to the first part of said series of cells, so as to apply the flotation agent to all parts of the pulp, by contact with said gas, and means for applying and distributing gas alone to a succeeding part of said series of cells, for aeration and flotation of the ore pulp therein.
5. The process of effecting froth-flotation separation, which consists in flowing an ore pulp into a cell having a porous bottom through which issues over a wide area an inert bubble-forming gas in small bubbles charged with a mineral-frothing agent in gaseous form, flowing the pulp also across a second porous bottom through which issues over a wide area an inert bubble-forming gas in small bubbles, substantially free from mineral-frothing agent, and separating the froth.
6. The process of effecting froth-flotation separation which consists in flowing an ore pulp into a cell having a porous bottom through which issues over a wide area an inert bubble-forming gas in small bubbles charged with a mineral-frothing agent in gaseous form, flowing the pulp also across a second porous bottom through which issues over a wide area an inert bubble-forming gas in small bubbles, substantially free from mineral-frothing agent, separating the froth, withdrawing the remainder of the pulp, flowing it over across another porous bottom through which issues over a wide area an inert bubble-forming gas in small bubbles, substantially free from mineral-frothing agent, and separating the froth.
7. The process of effecting froth-flotation separation which consists in flowing an ore pulp into a cell having a porous bottom through which issues over a large part of its width an inert bubble-forming gas in small bubbles charged with a mineral-frothing agent in gaseous form, separating the froth, flowing the remainder of the pulp into a cell having a porous bottom through which issues over a large part of its width an inert bubble-forming gas in small bubbles, substantially free from mineral-frothing agent, and separating the froth.
8. The process of effecting froth-flotation separation which consists in flowing an ore pulp through a cell with a porous bottom, forcing through a wide area of said bottom near the entrance of the ore pulp an inert bubble-forming gas in small bubbles charged with a mineral-frothing agent in gaseous form, also forcing an inert bubble-forming gas in small bubbles, substantially free from mineral-frothing agent, through a wide area of said bottom more remote from the entrance of the pulp, and separating the froth.
9. The process of effecting froth-flotation separation which consists in flowing an ore pulp through a cell with a porous bottom, forcing through a wide area of said bottom near the entrance of the ore pulp an inert bubble-forming gas in small bubbles charged with a mineral-frothing agent in gaseous form, also forcing an inert bubble-forming gas in small bubbles, substantially free from mineral-frothing agent, through a wide area of said bottom more remote from the entrance of the pulp, separating the froth, withdrawing the remainder of the pulp, flowing it through another cell with a porous bottom, forcing through a wide area of said bottom an inert bubble-forming gas in small bubbles, substantially free from mineral-frothing agent, through a wide area of said bottom, and separating the froth.
10. In a froth-flotation apparatus, the combination with cell walls, of a coarse porous bottom section adapted to admit a bubble-forming gas carrying a volatilized frothing agent, and a fine porous bottom section adapted to admit a bubble-forming gas, substantially free from mineral-frothing agent.
11. In a froth-flotation apparatus, the combination with cell walls, of means for admitting ore pulp, a coarse porous bottom section adapted to admit adjacent said means a bubble-forming gas carrying a volatilized mineral-frothing agent, and a fine porous bottom section more remote from said means adapted to admit a bubble-forming gas, substantially free from volatilized matter.

In testimony whereof I have hereunto subscribed my name this 27th day of October, 1917.

LEWIS BAILEY.